

## UNITED STATES PATENT OFFICE

2,371,710

## RESILIENT MATERIALS

George Schneider, Montclair, N. J., and Mervin E. Martin, Cumberland, Md., assignors to Celanese Corporation of America, a corporation of Delaware

No Drawing. Application November 12, 1941.  
Serial No. 418,861

3 Claims. (Cl. 288—34)

This invention relates to the preparation of resilient materials and relates more particularly to the production of resilient materials suitable for use as cushion liners in closures, such as those employed in the bottling industry.

An object of our invention is the preparation of resilient materials suitable for lining bottle closures, and the like, which are economical and highly efficient.

Another object of our invention is the preparation of artificial lining materials for bottle closures and the like which possess great flexibility as well as unusual resiliency.

Still another object of our invention is the preparation of lining materials for closures which materials are capable of maintaining an effective seal over wide fluctuations in the temperature and internal pressure of the contents of the containers on which they are applied.

Other objects of our invention will appear from the following detailed description.

Closures of various types are employed in sealing containers of glass or metal which are used for holding liquids. In the case of carbonated beverages such as soft drinks, beer, etc., where it is important to retain the gas in solution, the closures are usually in the form of a metal cap or shell lined with a disc of some soft, easily deformable material which may be covered with a flexible metal foil. The closures are put on the filled bottles by a suitable capping device which serves to bend the edges of the metal closure beneath a lip provided at the top of the bottle and to force the soft, foil-covered disc against the upper or pouring edge of the bottle. The pressure of the disc against the bottle acts as a seal and serves to prevent the escape of either the gas or the liquid. Ordinarily, the soft disc is formed of a material such as cork, but the quality and availability of this material varies from time to time. For this reason, a suitable material having the physical advantages of cork but which is readily available and whose quality can be controlled has long been sought.

We have now discovered that lining materials of unusual resiliency which are suitable for use as cushion liners for closures and capable of maintaining an effective seal when in use, may be prepared from cellulose fibers in sheet form, if the moisture content of said material is maintained at a relatively high level. In accordance with our invention, cellulose fibers compacted into the form of a sheet or web are so treated as to incorporate therein a hygroscopic material, and the sheet material then cut or

shaped in any convenient manner into discs or other shapes of suitable dimensions. The hygroscopic material incorporated into the sheet material maintains the moisture content of the discs at the desired relatively high level and thereby imparts to the latter an unusual degree of resiliency. The discs, when used alone, or more preferably, after being faced with a film or foil of a suitable inert material having a continuous structure, may then be used as cushion liners for lining container closures. The film or foil protects the sheet material from the action of the contents of the container. When the closures are applied by a suitable capping device, the cushion liners of our invention give a gas- and liquid-tight seal which remains tight through wide fluctuations in both the temperature and internal gas pressure of the container on which the closure is applied, as well as over extended periods of service.

Various hygroscopic materials may be employed for maintaining the moisture content of the cushion liners at the desired level and the hygroscopic materials, which may be liquid or solid, may be incorporated into said materials in many ways. The hygroscopic material may be incorporated into the cellulose fibers before they are formed into sheets, or the cellulose fibers may be treated after the sheets have already been formed. Preferably, the hygroscopic materials are applied after the fibers have already been fabricated into sheet form, or after the sheets have been cut or shaped into discs of the desired size. In this way, the amount incorporated therein may be more closely controlled and the moisture content may be maintained at any desired predetermined level by merely varying the relative amount of hygroscopic material used. Preferably, the moisture content is maintained at from 25 to 50% by weight. Examples of suitable hygroscopic material which may be employed are organic materials such as glycerine, glycols and sugars, or inorganic materials such as calcium chloride, magnesium chloride and sodium nitrate. The materials are preferably applied in solution in a suitable solvent such as, for example, water or ethyl alcohol. The hygroscopic materials may be employed in amounts varying from 15 to 50% on the weight of the cellulose fiber sheet material, but more or less may be incorporated, as stated, depending upon the particular moisture content desired for the particular application of the cushion liner.

The film or foil employed for facing the cellulose fiber cushion liner may be a separate film

or foil cut to the desired size and then placed in position, or the sheet material may be coated with a solution of a material in a volatile solvent which forms a film upon evaporation of said solvent. The film or foil over the face of the cushion liner prevents the liquid in the container from coming in contact with the cellulose fibers, as stated, and avoids any undesirable disintegration of said material whereby the fibers work loose to contaminate the beverage or other liquid in the container. The film or foil is preferably as inert as possible and may comprise a substance such as, for example, a film-forming derivative of cellulose, a polyvinyl condensation product, a film of regenerated cellulose, or a like material. The films are preferably unplasticized. Examples of cellulose derivatives which may be employed to form the films are cellulose esters such as cellulose acetate, cellulose propionate and cellulose butyrate, mixed esters such as cellulose acetate-propionate and cellulose acetate-butyrate, inorganic esters such as cellulose nitrate, and cellulose ethers, such as for example, ethyl cellulose and benzyl cellulose. Any suitable volatile solvent or mixture of solvents may be employed in forming a coating composition suitable for coating the sheet material used to form the cushion liner. Solvents such as, for example, acetone, chloroform, ethylene dichloride, acetone and ethyl or methyl alcohol, ethyl alcohol, and ethylene dichloride and ethyl or methyl alcohol are suitable.

The cellulose fiber cushion liner may be employed as a single layer of the desired thickness for lining the metal closures, or the cushion liner may comprise a plurality of layers sufficient to build up a layer of the desired thickness. The layers may be held in position as by some binding material or else the layers may be held in the metal closure merely by the pressure exerted when the cap or shell is applied to a container.

In order further to illustrate our invention but without being limited thereto the following examples are given:

#### Example I

Discs of suitable size are cut or punched from a compacted sheet of wood pulp cellulose of about 0.041 inch in thickness and the discs are then treated with a solution comprising equal parts by weight of glycerine and water. Two of these treated discs are chosen, inserted into a metal closure of the cap type in register and faced with a cellulose acetate film about 0.004 inch in thickness. The assembled closure is then applied to a bottle holding a carbonated beverage by means of a capping device. The sealed bottles are then subjected to a pasteurization treatment during which the internal pressure rises from the usual 35 pounds per square inch to 100 pounds per square inch. On cooling, the pressure returns

to 35 pounds per square inch and remains there. The seal formed by the cellulose disc remains permanently tight and there is no loss in pressure due to the escape of gas.

5

#### Example II

Wood-pulp cellulose discs of proportions similar to those of Example I are prepared, inserted into a bottle cap in register, and faced by an un-plasticized cellulose acetate film 0.004 inch in thickness, the whole system being cemented together by small quantities of cellulose acetate solution in acetone. There is then added around the edges of the seal an amount of 50%-50% diethylene glycol-water mixture equal to the weight of wood-pulp cellulose. The cap is allowed sufficient time to equalize the concentration of hygroscopic material before capping, 1 to 2 hours being usually sufficient. The assembled closure

10

is then applied to a bottle by a capping device and the resulting seal remains tight to gas and liquid under the varying conditions of temperature and pressure during pasteurization as well as after.

15

It is to be understood that the foregoing detailed description is given merely by way of illustration and that many variations may be made therein without departing from the spirit of our invention.

20

Having described our invention, what we desire to secure by Letters Patent is:

1. A resilient material adapted to be employed to form a pressure seal, comprising a compact material in sheet form having a basis of wood-pulp cellulose fibers and having incorporated therein an aqueous solution containing from 15 to 50% of an organic hygroscopic material selected from the group consisting of glycerine and diethylene glycol, and a facing of a preformed organic derivative of cellulose foil secured to said material.

25

2. A resilient material adapted to be employed to form a pressure seal, comprising a compact material in sheet form having a basis of wood-pulp cellulose fibers and having incorporated therein an aqueous solution containing from 15 to 50% of an organic hygroscopic material selected from the group consisting of glycerine and diethylene glycol, and a facing of a preformed cellulose acetate foil secured to said material.

30

3. A resilient material adapted to be employed to form a pressure seal, comprising a compact material in sheet form having a basis of wood-pulp cellulose fibers and having incorporated therein an aqueous solution containing 50% of an organic hygroscopic material selected from the group consisting of glycerine and diethylene glycol, and a facing of a preformed cellulose acetate foil secured to said material.

35

GEORGE SCHNEIDER.  
MERVIN E. MARTIN.